

# UNITED STATES PATENT OFFICE.

OLE ROLFSEN, OF LARVIK, NORWAY.

## LUBRICANT OIL.

No Drawing. Application filed June 17, 1928, Serial No. 116,619, and in Norway March 12, 1925.

This invention has for its object a lubricant which is particularly suitable for automobile engines and other combustion- or explosion engines especially in such systems in which the engine cylinder oil is also used for the lubrication of bearings and gears.

This lubricant substantially consists of mineral oil with an addition of fatty acid glycerides of marine origin.

10 As compared with known lubricants containing fatty acid glycerides as an addition the present lubricant is distinguished in that it contains an incompletely hydrogenized whale oil containing considerable proportions of saturated as well as unsaturated fatty acid glycerides.

The whale oil product to be used as an addition to the mineral oil can be obtained by any of the known methods of hydrogenating 20 oils by blowing with hydrogen in the presence of catalysts.

While the hydrogenation treatment is continued only to the point at which the product is of a pasty or semi-fluid character at ordinary temperature, the percentage of unsaturated fatty acid glycerides will be sufficiently high to comply with the requirements of the invention.

For example, 100 kilograms of whale oil 30 with an iodine number of about 110 is freed from soluble albumen and dirt by treatment with sulphuric acid as is usual in this art

and then dried in a vacuum at a temperature not exceeding 90° C. To this oil is added about 2 kilograms of nickel-on-kieselguhr 35 catalyst and containing about .5 kilograms of metallic nickel. The oil is then placed in a hydrogenation apparatus, hydrogen injected and the temperature raised to about 160° C. When about 3 cubic meters of 40 hydrogen have been absorbed by the charge the hydrogen is shut off, the charge cooled and the catalyst separated out by means of a filter press. The resulting incompletely hydrogenated oil is then mixed with from 45 2500-3000 kilograms of mineral oil to form the compounded lubricant.

The proportion of partially hardened oil which has to be added to the mineral oil will vary according to the conditions under 50 which the lubricant is to be used, the character or duration of the hydrogenation treatment and of the initial materials employed.

### Claims:

1. A lubricant comprising a mineral oil 55 and a substantial proportion of an added incompletely-hydrogenated whale oil.
2. A lubricant comprising a mineral oil, and between 5-10% of an added incompletely-hydrogenated whale oil. 60

In testimony whereof I have signed my name to this specification.

OLE ROLFSEN.